

July 21 1925.

1,546,937

S. B. MATHEWSON ET AL

CARBONIZING COMPOUND AND PROCESS OF MAKING AND USING IT

Original Filed April 3, 1922



INVENTORS  
Walter K. Garrison  
Stanley B. Mathewson

Paulin Paulin,  
ATTORNEYS

## UNITED STATES PATENT OFFICE.

STANLEY B. MATHEWSON, OF SPRINGFIELD, AND WALTER K. JAMISON, OF DAYTON, OHIO, ASSIGNEES TO WALTER K. JAMISON, STANLEY B. MATHEWSON, HOWARD F. MARSTON, (MRS.) W. K. JAMISON, AND (MRS.) S. B. MATHEWSON, TRUSTEES OF THE LECAR CARBON COMPANY, OF SPRINGFIELD, OHIO, A TRUST ESTATE.

## CARBONIZING COMPOUND AND PROCESS OF MAKING AND USING IT.

Original applications filed April 3, 1922, Serial No. 549,274, and August 7, 1922, Serial No. 580,225. Divided and this application filed December 6, 1923. Serial No. 678,986.

To all whom it may concern:

Be it known that we, STANLEY B. MATHEWSON and WALTER K. JAMISON, citizens of the United States, residing at Springfield, Clark County, Ohio, and Dayton, Montgomery County, Ohio, respectively, have invented certain new and useful Improvements in Carbonizing Compounds and Processes of Making and Using Them, of which the following is a specification, reference being had therein to the accompanying drawing.

Our invention relates to a carbonizing compound and the process of making it and using it for carbonizing metal, and in particular case hardening steel. The object of our invention is to utilize scrap leather by the treatment of our invention hereinafter described and claimed.

An additional object of our invention is to provide a new product by this treatment which may be utilized as a carbonizing material.

It is a further object of our invention to provide a method of utilizing our new product in case hardening metals such as steel in order to provide a very deep case in the minimum of time and economically.

This is a division of applications No. 549,274, filed Apr. 3, 1922, and 580,225, filed Aug. 7, 1922.

Referring to the drawings:

Fig. 1 is a carbonizing can;

Fig. 2 is a diagrammatic view of the furnace in which the carbonizing can is placed with the scrap leather in order to reduce it to the form of the product now in question;

Fig. 3 is a diagrammatic view of the rolls and screen for determining the size and grade of the resulting carbonized product;

Fig. 4 is an end elevation of a piece of steel before treatment with this carbonizing material;

Fig. 5 is a similar view after carbonization showing the case;

Fig. 6 is a section of a carbonizing box packed with the carbonizing material involved herein showing the articles being

carbonized and the arrangement of their packing.

It will be understood that the foregoing drawings are diagrammatic merely and are only for the purpose of illustration.

Referring to the drawings in detail, 1 is a carbonizing can or metal container having a lid 2 with apertures 3 in the lid thereof. The scrap leather is placed in this can and the can is placed in an oven 4. This oven is heated by any desired means as for instance by burners such as at 5. It will be understood that this illustration of the burners is typical only and that any kind of heating apparatus may be employed. The cans are sealed and the lids are tight fitting. The openings 3 are provided in the cans to permit of the adjustment of the internal pressure and to permit of the escape of gases within the container.

The cans are preferably packed in an oil furnace, the temperature of which has been brought up to 1200 degrees F., at which time the burners are shut off and the furnace sealed with the exception of the regular ventilation therefor. It is customary to allow the furnace to remain closed for about six hours, after which time the containers can be removed and the finished product may be removed from each one of the individual containers. It is then crushed between the rollers 6—6 and screened by the screen 7 which is preferably about of a  $\frac{3}{8}$ " mesh. The purpose of this is to reduce it to a suitable size for carbonizing purposes.

## Process of hardening steel.

The finished product thus secured is used as follows: The parts to be carbonized are thoroughly cleansed in an alkali solution in order to remove all dirt and oil. Any cleansing solution of similar character may be employed. They are then packed in the boxes 8 so that the parts 9 will be arranged in layers in the carbonizing material 10. The top of the box is sealed with fire clay as at 11. It is the preferred practice to place a layer of the carbonizing material, then a layer of parts separated from one

another by the carbonizing material, a layer of carbonizing material and another layer of parts, and so on. The whole packing is covered with a layer of the carbonizing material.

If desired the lid may be of metal and sealed with fire clay. Any common practice of this sort may be followed. The boxes are then placed in a carbonizing furnace and the 10 temperature brought up to 1700 degrees F. and held at this temperature for about three hours, but this time and temperature varies upon the depth of case desired, the size of the parts to be carbonized and the size of the 15 carbonizing boxes.

In the event the furnace is cold when the boxes are placed therein a proportionately greater time will be necessary to effect the desired result.

20 The boxes employed are usually about eight and one-half inches in diameter, eleven inches deep and walls about  $\frac{3}{8}$ " thick. It takes about three hours to bring a packed box up to the temperature of 1700 degrees, 25 the temperature used for carbonizing.

For instance, in the case of carbonizing S. A. E. 10-20 steel, it has been found good practice with this carbonizing material to hold the carbonizing heat at 1700 degrees F. 30 for five hours when packed in a box of the above mentioned dimensions in order to obtain a  $\frac{1}{2}$ " depth of case.

The preferred method after this temperature has been maintained this desired length 35 of time is to allow the case hardened steel parts to cool in the carbonizing boxes before they are exposed to the air.

We do not desire to confine our invention to any particular type of furnace for the 40 heat treatment. An open type furnace may be employed in which the temperature has been brought up to 1450 degrees F. before the parts are placed in the furnace. It will then customarily require about fifteen to 45 twenty minutes to bring a  $\frac{3}{4}$ " part, speaking in terms of diameters, up to 1450 degrees. The parts are then removed and quenched in brine or oil. It will be understood that these parts are always removed 50 from the furnace and quenched on the rising heat.

In the second method a salt bath may be used and the parts are immersed in this solution. After the solution has been 55 brought up to 1450 degrees F. the parts are removed and quenched in brine or oil. This type of furnace is usually designated a cyanide furnace. It will be understood that the fire does not come in direct contact with 60 the work as a cast iron tank is placed in the furnace and the salt solution is placed in the tank and melted by the heat coming in contact with the outside of the tank.

65 It will be further understood that it is preferred by us that all quenching solutions

be retained as at low a temperature as possible, which is accomplished by any well known means such as circulating the solution through cooling coils.

Referring to Figs. 4 and 5, 12 is a specimen of steel and 13 is the case.

When the carbonizing material so produced by the above mentioned process is examined with the naked eye it appears to be a porous cellular structure with a highly 75 vitrified appearance. The apertures therein and therethrough are irregular in shape and size.

The carbonaceous material referred to herein as the carbonizing compound is generally composed of approximately 30% to 31% volatile matter, about 3% moisture, about 58% fixed carbon and about 8% ash.

It will be understood that these amounts are approximate.

Upon analysis the ash will usually develop a ferric oxid color. The volatile matter consists of various gases. In these gases a varying amount of ammonia will be found and the usual reaction to litmus will be alkaline.

While we have shown and described certain features as constituting our invention, it will be understood that parts have been shown for purposes of illustration only, and 95 that we do not desire to be limited to such details, as obvious modifications will occur to persons skilled in the art.

Having thus fully described our invention, what we claim as new and desire to secure by Letters Patent, is:—

1. In a method of producing a carbonizing material, placing scrap leather and the like in a receptacle closed except for small 105 holes in it, placing a receptacle in a furnace and heating the receptacle therein, allowing the receptacle and its contents to cool, sealing the furnace except for natural draft and allowing the furnace to cool with the boxes therein for a predetermined 110 period.

2. In a method of producing a carbonizing material, placing scrap leather and the like in a partially sealed receptacle in a furnace and heating the receptacle therein, allowing the receptacle and its contents to cool, sealing the furnace except for natural draft and allowing the furnace to cool with the boxes therein for a predetermined period, 115 removing the boxes, crushing the material and screening it.

3. In a process of producing a carbonizing material, placing scrap leather and the like in partially sealed containers having apertures in the top thereof for the exit of gases therefrom, placing the containers in a furnace, heating the containers for a predetermined period, allowing the receptacle and its contents to cool but allowing the container to remain within the furnace a pre- 125

determined period and removing the containers and the material therefrom.

4. In a process of producing a carbon material, placing scrap leather in a receptacle which is sealed save for a vent, heating until the temperature is brought up to 1200 degrees Fahrenheit, sealing the furnace and allowing it to remain closed for about six hours, and opening the furnace and removing the material from the container.

5. In a process of producing a carbon material, placing scrap leather in a partially sealed container, heating it until it reaches a temperature of about 1200 degrees Fahrenheit, sealing the furnace in which the container is located and allowing the container and its contents to cool, allowing a portion of the gases generated to escape during the heating period and allowing the remainder of the gases generated to be reabsorbed by the material upon cooling, whereby the material upon completion will have the appearance of a granular mass or of a vitrified sponge, consisting of about 60 per cent carbon, 30 to 40 per cent volatile matter in suspension, and the remainder in moisture and ash.

6. In a process of producing a carbon

material, treating scrap leather by heating it to a predetermined temperature, generating gases from it during the heating period partially confining the generated gases and allowing the mass to cool to reabsorb said gases while cooling, whereby a resulting compound is produced, consisting of carbon and nitrogen products in suspension therein adapted to be released upon the heating of the product to a predetermined temperature.

7. In a process of producing a carbon material, treating scrap leather by heating it to a predetermined temperature, generating gases from it during the heating period partially confining the generated gases and allowing it to cool to reabsorb said gases while cooling, whereby a resulting compound is produced, consisting of carbon and nitrogen products in suspension therein adapted to be released upon the heating of the product to a predetermined temperature, said carbon consisting of about 60 per cent of the product and the nitrogenous products consisting of about 30 to 40 per cent of the product.

In testimony whereof we affix our signatures.

STANLEY B. MATHEWSON.

WALTER K. JAMISON.